

No. 650,861.

Patented June 5, 1900.

T. J. McTIGHE.

ELECTRICAL CONNECTOR AND METHOD OF MAKING SAME.

(Application filed Mar. 30, 1900.)

(No Model.)



Witnesses  
S. McTighe  
Lest McTighe

Thomas J. McTighe  
Inventor

By his Attorney, Connelly Bros.

# UNITED STATES PATENT OFFICE.

THOMAS J. MCTIGHE, OF NEW YORK, N. Y.

## ELECTRICAL CONNECTOR AND METHOD OF MAKING SAME.

SPECIFICATION forming part of Letters Patent No. 650,861, dated June 5, 1900.

Application filed March 30, 1900. Serial No. 10,838. (No model.)

*To all whom it may concern:*

Be it known that I, THOMAS J. MCTIGHE, a citizen of the United States, residing at New York, in the county of New York and State 5 of New York, have invented certain new and useful Improvements in Electrical Connectors and Methods of Making the Same; and I do hereby declare the following to be a full, clear, and exact description of the invention, 10 such as will enable others skilled in the art to which it appertains to make and use the same.

This invention relates to the manufacture of electric-railway-rail bonds, especially of that class wherein the terminals or rail-attaching studs are fixed on the extremities of a flexible connector consisting of a number of separate wires or bars or a piece of ordinary wire cable, such terminals and connector being usually of copper. As it is desirable that 20 there should be no appreciable resistance between the connector and its terminals, various plans have been adopted to secure a close contact. The ends have been placed in a mold and molten copper poured in to fill 25 around the connector and form the stud, and while both terminal and connector are at a high temperature a drop-hammer is applied to consolidate the parts together. Another plan is to form the terminals first, by casting 30 or otherwise, then insert the cable or connector, bring both up to a welding temperature, and then press them into a substantially-welded condition. In all methods involving 35 the application of heat the high temperature causes the rapid formation of oxid on the connector itself, thus appreciably reducing its conductivity, and it practically prohibits the use of insulation on the connector.

In practicing my invention I do not raise 40 the temperature of the cable or connector, but effect the union of the parts cold, thus avoiding oxidation and obtaining a number of advantages.

To this and other ends my invention consists in the manufacture of electric connecting devices—such as railway-rail bonds, dynamo-terminals, &c.—by swaging the parts together by great pressure applied cold, substantially as hereinafter fully described and 45 claimed.

In the drawings which form part of this

specification, Figure 1 is a sectional view of the dies and plunger of a press adapted to carry out my invention, the parts being shown ready to receive one end of a rail-bond and 55 cold-swage the same. Fig. 2 is a top view of the lower die with the terminal therein. Fig. 3 is a much-enlarged cross-section of the rail-bond on the line *x* *x* of Fig. 2 after the cold-swaging. Fig. 4 shows a plan and edge view 60 of a dynamo-terminal with cable-socket. Fig. 5 shows a plan and edge view of the same with the cable inserted and the two cold-swaged together. Fig. 6 shows an edge and plan view of a bus-bar coupling or clamp and 65 flexible connector cold-swaged together.

For making rail-bonds I use a shaping-die A, a confining-die B, and a plunger C. The precise shape of the working parts of these will depend upon the shape to be given the 70 terminal. I show one end of a rail-bond composed of the rail-attaching stud *d*, its head *e*, and the flexible cable *f*.

The confining-die B may have a cavity *g* cut in it, as shown, for forming part of the 75 head *e*, or the shoulder-cavity *h* may be recessed deeply enough in the die A to avoid making any cavity in the die B. The die A has a hole *i* bored through it, the lower portion being tapered to facilitate withdrawal of 80 the pressed terminal. The plunger C is arranged to enter the hole *i* and, if desired, may be attached to the platen of the press.

I take a cast or drop-forged copper terminal approximating the desired finished form, 85 as shown in Fig. 1, having a hole or socket formed in it transversely to receive the end of the terminal *f*. This hole may be round; but I prefer a flattened or elliptical form, as shown. I prefer to clean the terminal with 90 acid or otherwise and remove all oxid or scale and dirt from the surface, leaving the latter bright and untarnished. The end of the cable *f* is then inserted in the hole, as shown in Fig. 1, and the dies are brought together, 95 after which great pressure is applied by means of the plunger C, actuated by a suitable press. This presses upon the end of the stud *d*. As the pressure increases the metal of the terminal is compelled to flow and fill 100 all the cavities in the mold or die, consolidating the whole mass of the wires of cable *f* in

and with the head *e* and the stud *d*. By this method of swaging cold and under great pressure I produce a close union of the wires of the cable with the terminal *d e*, an effect which I call "cold welding." The effect of the great pressure is illustrated in Fig. 3, where it is seen that the metal of the terminal fills the external crevices of the cable, the voids in the cable have been eliminated, and the originally-round wires are pressed into hexagonal shape, bringing all the surfaces into such intimate and cohesive contact as to constitute a weld for the purposes intended and without the possibility of oxidation or "burning" by overheating.

While the invention is thus designed and shown as especially applicable to the manufacture of rail-bonds, various other electrical applications come within its scope. For example, Figs. 4 and 5 illustrate it as applied to dynamo-terminals. For large generators the connections between the movable brush-holders and the stationary connection-board of the machine are usually made of very flexible cable, and the cable is covered with insulation. The terminals are usually attached by soldering, with resulting imperfect and uncertain conductivity and damage to the insulation by heat. I make such a terminal *T* of soft copper, with the socket *s*, into which the end of the cable *f'* is inserted, and then by using appropriate dies and great pressure I swage the whole mass into the above-described condition of a "cold weld," as in Fig. 5, affording perfect conductivity without injury to the insulation on the remainder of the cable.

In Fig. 6 I show the same method applied to the socket *m* of a clamp *n* for attaching a branch cable *f''* to the bus-bar *P* of a switch-board. In practice I find that a pressure of about one hundred thousand pounds per

square inch is well adapted to effect the desired result.

As compared with the usual soldered connection my cold-welded terminals have the important advantage that under an overload of electric current there is no solder to melt and run out and make trouble.

Having described my invention, I claim as new and desire to secure by Letters Patent—

1. The method of uniting an electrical conductor to a metallic terminal, which consists in inserting one into the other and cold-welding them together by pressure.

2. The method of uniting an electrical conductor to a metallic terminal, consisting in inserting one into the other and cold-swaging them into mutually-coherent homogeneous masses.

3. The method of uniting an electrical conductor to a metallic terminal, consisting in inserting the conductor into the terminal and swaging the two together under pressure sufficient to cold-weld the contacting surfaces.

4. The method of manufacturing rail-bonds, consisting in fitting the ends of a flexible conductor into suitably-shaped terminals and swaging the parts together under pressure sufficient to cold-weld the contacting surfaces.

5. An electrical connection composed of a suitably-shaped terminal and a flexible conductor swaged and cold-welded together.

6. A rail-bond consisting of a flexible conductor and terminals having shoulders and attaching-studs, said terminals and conductor being swaged and cold-welded together.

In testimony whereof I affix my signature in presence of two witnesses.

THOMAS J. MCTIGHE.

Witnesses:

THOS. A. CONNOLLY,  
Jos. B. CONNOLLY.